

## UNITED STATES PATENT OFFICE

2,191,813

ELECTRODEPOSITION OF NICKEL FROM  
AN ACID BATH

Henry Brown, Detroit, Mich., assignor to The  
Udylite Corporation, Detroit, Mich., a corpora-  
tion of Delaware

No Drawing. Application December 1, 1939,  
Serial No. 307,060

31 Claims. (Cl. 204—14)

This invention relates to the electrodeposition of nickel from an acid bath.

The object of this invention is to decrease the grain size and increase the lustre of the nickel deposit without decreasing appreciably the ductility of the plate or the current density range of the nickel bath.

I have found that this object can be accomplished by the addition of certain organic compounds to the standard nickel plating baths. The compounds are the ones which contain the sulphonamide or sulphonimide group  $-\text{SO}_2\text{N}=$ .

In table I are listed a number of compounds containing the sulphonamide or the sulphonimide group which produce the result sought to be achieved provided the compound is soluble in the nickel solution. These organic sulphonamides and sulphonimides contain in common the  $-\text{SO}_2\text{N}=$  group. They may be classified as compounds containing the  $-\text{SO}_2\text{N}=$  group. These organic sulphonamides and sulphonimides contain in common the  $-\text{SO}_2\text{N}=$  group attached to carbon linked by the alternate double bond sequence constituting the nucleus of the aromatic series. These compounds may, therefore, also be classified as containing in common the



group. This structure, for example, is present in:

35 1. Benzene sulphonamide



45 2. o-Benzoic sulphonimide



3.  $\beta$ -naphthalene sulphonamide



The strength of the bond between the carbon and sulphur linkage appears important. It is modified by other active groups present and the rest of the structure of the molecule. For example,  $\alpha$  naphthalene sulphonamide gives much greater brightness and over a wider current density range than an equal concentration of  $\beta$ -naphthalene sulphonamide. The odor of naphthalene is apparent at the cathode with  $\alpha$  naphthalene sulphonamide, but is not apparent with the beta compound. In fact the alpha derivative is somewhat too active and unstable during electrolysis for best practical results. This result is in keeping with the generally greater stability of other beta naphthalene derivatives compared to the alpha, and their general and rather striking differences in chemical properties. The benzene series of sulphonamides as to be expected, shows greater regularity, and the brightening action is more commensurate with the solubility of the compound in the nickel bath. In general, the greater the concentration of the compound, the wider is the current density range in which the brightening action is produced. With the less soluble (0.5 g./l. or less) sulphonamides, such as  $\beta$  naphthalene sulphonamide, p-toluene sulphonmethylamide, pp' biphenyl disulphonamide, benzene metadisulphonamide, the brightening action is manifested mainly in the lower current density areas, whereas the more soluble compounds show their brightening action at all plating current densities. Therefore, from the practical standpoint, it is preferred to use the more soluble compounds such as benzene sulphonamide, o- and p-toluene sulphonamide and o-benzoic sulphonimide. In general, these compounds can be used up to saturation to give beneficial results. However, all of these compounds even with concentrations in the neighborhood of 0.1 g./l. produce the desired results at the low current densities; therefore, even the slightly soluble compounds produce desirable results.

Table I also contains the optimum concentra-

tions of the various compounds in suitable nickel solutions such as listed in Table II.

Table I

|    |                                                                                                                  |                                             |
|----|------------------------------------------------------------------------------------------------------------------|---------------------------------------------|
| 5  | Benzene sulphonamide, $C_6H_5SO_2NH_2$                                                                           | 1-3 g./l. (sat.)                            |
|    | $\text{O}-\text{Benzoyl sulphonimide, } \text{NH}-\text{C}_6\text{H}_4\text{CO}$                                 | 1-2 g./l.                                   |
|    | p-Benzoic sulphonamide, $\text{HOOC-C}_6\text{H}_4\text{SO}_2\text{NH}_2$                                        | .5-1 g./l. (sat.)                           |
| 10 | o- or p-Benzoic sulphonodichloramide, $\text{HOOC-C}_6\text{H}_4\text{SO}_2\text{NCl}_2$                         | .5-1 g./l. (sat.)                           |
|    | p-Toluene sulphonamide, $\text{C}_6\text{H}_5\text{CH}_2\text{SO}_2\text{NH}_2$                                  | 1.0-3 g./l. (sat.)                          |
|    | o-Toluene sulphonamide, $\text{C}_6\text{H}_5\text{CH}_2\text{SO}_2\text{NH}_2$                                  | 1.0-2 g./l. (sat.)                          |
|    | p-Toluene sulphonchloramide, $\text{C}_6\text{H}_5\text{CH}_2\text{SO}_2\text{NHCl}$                             | 1-3 g./l. (sat.)                            |
| 15 | Sodium p-toluene sulphonchloramide, $\text{C}_6\text{H}_5\text{CH}_2\text{SO}_2\text{NNaCl}_3\text{H}_2\text{O}$ | 1-4 g./l.                                   |
|    | p-Toluene sulphonodichloramide, $\text{C}_6\text{H}_5\text{CH}_2\text{SO}_2\text{NCl}_2$                         | Insoluble, OK as it loses Cl                |
|    | p-Toluene sulphonmethylamide, $\text{C}_6\text{H}_5\text{CH}_2\text{SO}_2\text{NHCH}_3$                          | Very slightly soluble and has slight effect |
|    | p-Toluene sulphonethylamide, $\text{C}_6\text{H}_5\text{CH}_2\text{SO}_2\text{NHCH}_3$                           | Insoluble                                   |
| 20 | p-Brom benzene sulphonamide, $\text{C}_6\text{H}_5\text{BrSO}_2\text{NH}_2$                                      | .5 g./l. (sat.)                             |
|    | p,p'-Diphenyl disulphonamide, $\text{NH}_2\text{SO}_2\text{C}_6\text{H}_4\text{SO}_2\text{NH}_2$                 | .5 g./l. (sat.)                             |
|    | Benzene meta disulphonamide, $\text{C}_6\text{H}_4\text{(SO}_2\text{NH}_2)_2$                                    | .5 g./l. (sat.)                             |
|    | $\alpha$ -naphthalene sulphonamide, $\text{C}_10\text{H}_7\text{SO}_2\text{NH}_2$                                | .25 g./l.                                   |
| 25 | $\beta$ -naphthalene sulphonamide, $\text{C}_10\text{H}_7\text{SO}_2\text{NH}_2$                                 | .5 g./l. (sat.)                             |

ductile and adherent coating can be obtained and within wider current density limits, upon which chromium may easily be applied. The sulphonamides or sulphonimides also decrease the sensitivity of the plating to otherwise harmful concentrations not only of zinc and cadmium but to such other ions that may plate out or be included in the plate such as copper, arsenic, selenium, tellurium and mercury. The sensitivity to small amounts of harmful organic colloids which may cause poor bond and brittle plate is also decreased. Therefore, a nickel coating which peels off on bending due to the presence of buffing dirt in the bath, will adhere after the addition of a soluble sulphonamide or sulphonimide to the bath. This does not mean, however, that a still larger excess of colloid would not be harmful or even exceedingly harmful, but that the harmful effects are not as critical as in the absence of the sulphonamides. It was observed, for example, that the covering power in deep recesses (low current density areas) of a hot Watts bath freshly made up from commercial nickel salts was improved by the addition of toluene sulphonamide. This shows in another way its effect upon impuri-

Table II

| 30 | Bath No. | NISO <sub>4</sub><br>7H <sub>2</sub> O<br>g./l. | NiCl <sub>2</sub><br>6H <sub>2</sub> O<br>g./l. | Buffer                                                          |        | Other salts                          |       | Temp.,<br>°F. | pH  | Current density,<br>amps./sq.<br>ft. | 30 |
|----|----------|-------------------------------------------------|-------------------------------------------------|-----------------------------------------------------------------|--------|--------------------------------------|-------|---------------|-----|--------------------------------------|----|
|    |          |                                                 |                                                 | Formula                                                         | g./l.  | Formula                              | g./l. |               |     |                                      |    |
| 35 | 1        | 300                                             | 45                                              | H <sub>3</sub> BO <sub>3</sub> (boric acid)                     | 40     |                                      |       | 75-160        | 2-6 | 10-75                                | 35 |
|    | 2        | 300                                             | 45                                              | H <sub>3</sub> BO <sub>3</sub>                                  | 30     |                                      |       | 75-160        | 1-5 | 10-100                               |    |
|    | 3        | 75                                              | 225                                             | H <sub>3</sub> BO <sub>3</sub>                                  | 35     |                                      |       | 75-160        | 2-6 | 10-85                                |    |
|    | 4        | 300                                             | 45                                              | H <sub>2</sub> COOH (formic acid)                               | 35     |                                      |       | 75-140        | 3-6 | 10-60                                |    |
| 40 | 5        | 200 to 300                                      | 45                                              | H <sub>3</sub> BO <sub>3</sub>                                  | 4 to 8 |                                      |       | 75-140        | 2-6 | 10-60                                | 40 |
|    |          |                                                 |                                                 | NiF <sub>2</sub>                                                |        |                                      |       |               |     |                                      |    |
|    |          |                                                 |                                                 | or                                                              |        |                                      |       |               |     |                                      |    |
|    |          |                                                 |                                                 | H.F.                                                            | 2 to 4 |                                      |       |               |     |                                      |    |
|    | 6        | 300                                             | 45                                              | C <sub>6</sub> H <sub>5</sub> O <sub>2</sub> COOH (furoic acid) | 30     |                                      |       | 75-140        | 3-6 | 10-60                                |    |
|    | 7        | 300                                             | 45                                              | H <sub>3</sub> BO <sub>3</sub>                                  | 40     | MgSO <sub>4</sub> ·7H <sub>2</sub> O | 125   | 75-160        | 2-6 | 10-60                                |    |
|    | 8        | 75                                              |                                                 | (Na-citrate)                                                    | 15     | NaCl                                 | 40    | 75            | 5.5 | 10-25                                |    |
|    | 9        | 75                                              |                                                 | H <sub>3</sub> BO <sub>3</sub>                                  | 15     | (NH <sub>4</sub> Cl)                 | 15    | 75            | 5.5 | 10-25                                |    |
|    | 10       | 100                                             |                                                 | H <sub>3</sub> BO <sub>3</sub>                                  | 15     | (Na <sub>2</sub> SO <sub>4</sub> )   | 75    | 75            | 5.3 | 6-20                                 |    |
|    |          |                                                 |                                                 |                                                                 |        | NH <sub>4</sub> Cl                   |       |               |     |                                      |    |

55 These addition agents are preferably used in the type of grey-nickel bath which produces ductile, soft, adherent nickel deposits of any thickness. The baths should preferably be capable of operating warm in order to obtain higher conductivity and therefore higher current densities. Baths Nos. 1-7 in Table II are typical of nickel plating baths of preferred formulations.

55 The additions of small quantities of zinc and cadmium ions to the nickel solutions containing the sulphonamides produce a very marked increase in the rate of brightening and lustre. While cadmium and zinc salts have been used previously as "brighteners" in plain nickel solutions without the organic addition agents mentioned here, they have not proved generally successful especially where heavier thicknesses of nickel were demanded. The slightest excess of these ions caused dark streaks in the plate and skipping of plate in the recesses or low current density areas. Furthermore, the brightest plates obtained are very hard and brittle, and if plated to a thickness of .0005" and over as required by today's specifications, the danger of peeling of the coating is very great, especially with the subsequent application of chromium plate over such nickel coatings where the additional stress will cause the coating to crack and lift from the basis metal.

75 The presence of the sulphonamides changes these conditions, and a much brighter and more

ties which are the cause of the poor color or lack of plate in the recesses.

The presence of sodium and ammonium salts is not desirable as a general rule. However, the sulphonamides alone can be used with beneficial effects in any nickel plating bath that is giving satisfactory commercial plates for any given purpose, such as baths 8 through 10 in Table II. In the presence of zinc or cadmium ions the sodium and ammonium salts give rise to more brittle and poorly adherent plate. Vice-versa, less zinc or cadmium is tolerated in the presence of sodium or ammonium ions. For example, while 3 to 4 g./l. of Na<sub>2</sub>SO<sub>4</sub> or (NH<sub>4</sub>)<sub>2</sub>SO<sub>4</sub> produce no appreciable harm when maximum allowable zinc or cadmium is present, much higher concentrations will produce hard, brittle, poorly adherent plate of poor color and which stain easily. This is much more marked in the warm baths. Sodium salts are less critical than ammonium salts and magnesium salts are much less critical.

75 The best buffers are boric and formic acids. Furoic acid and fluoboric acid may be used, but acetic and citric are not recommended because they interfere with the brightness of the deposit.

The preferred baths Nos. 1-7 listed in Table II are operated with 1-3 g./l. of benzene sulphonamide or p-toluene sulphonamide or others of the more soluble sulphonamides or a mixture of two. The concentration of zinc or cadmium that can be used with the sulphonamide will depend

- on the temperature and the pH of the bath, concentration of nickel ions, concentration of buffer, and to a certain extent on type of sulphonamide or sulphonimide. In general, up to about 0.3 g./l. of zinc or up to about .4 g./l. of cadmium may be used in warm baths 1 to 7 listed in Table II. The usual operating temperatures are 100-160° F. and at pH values of 2.5-4.5. The lower pH values are used with higher temperatures.
- 10 The sulphonamides produce bright nickel plate over smooth buffed basis metals, such as buffed brass, and the nickel plate needs no subsequent buffing even when plated several thousandths of an inch thick.
- 15 The various sulphonamides and sulphonimides are mutually compatible and mixtures can be employed in the baths often to an advantage.
- This application is a continuation in part of application Serial No. 162,696, filed September 7, 20 1937.
- I claim:
1. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, in the presence of a compound soluble in the acid nickel solution and containing the group  $-\text{SO}_2\text{N}-$ .
2. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, in the presence of a compound containing the group  $-\text{SO}_2\text{N}-$ , which compound is soluble in the solution and has a concentration in the acid nickel solution falling within the range from .1 gram per liter of solution to saturation.
3. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, having a pH falling within a range of from about 2 to about 6 electrometric in the presence of a compound containing the group  $-\text{SO}_2\text{N}-$ , which compound is soluble in the solution and has a concentration in the solution falling within a range of .1 gram per liter of solution to saturation.
4. A method for electrodepositing nickel to obtain a fine grained lustrous deposit comprising the step of electrodepositing nickel from an aqueous acid nickel solution comprising essentially nickel sulphate, nickel chloride and boric acid having a pH falling within a range of from about 2 to about 6 electrometric in the presence of a compound containing the group  $-\text{SO}_2\text{N}-$ , which compound is soluble in the solution and has a concentration in the solution falling within a range of .1 gram per liter of solution to saturation.
5. A method for electrodepositing nickel to obtain a fine grained lustrous deposit comprising the step of electrodepositing nickel from an aqueous acid solution comprising essentially nickel sulphate, nickel chloride and boric acid containing about 60 to 75 grams per liter of nickel, about 15 grams per liter of chloride, about 30 to 37.5 grams per liter of boric acid, and having a pH falling within a range from about 2 to about 6 electrometric in the presence of a compound containing the group  $-\text{SO}_2\text{N}-$ , which compound is soluble in the solution and is present in the solution in amounts falling within a range from about .1 gram per liter of solution to saturation.
6. A method for electrodepositing nickel to obtain a fine grained lustrous deposit comprising the step of electrodepositing nickel from an aqueous acid nickel solution comprising essentially boric acid and a material selected from the group consisting of nickel sulphate, nickel chloride, and a mixture of nickel chloride and nickel sulphate, in the presence of a compound soluble in the acid nickel solution and containing the group  $-\text{SO}_2\text{N}-$  and in the presence of a cadmium salt in an amount corresponding to less than about .4 gram cadmium per liter of solution.
7. A method for electrodepositing nickel to obtain a fine grained lustrous deposit comprising the step of electrodepositing nickel from an aqueous acid nickel solution comprising essentially boric acid and a material selected from the group consisting of nickel sulphate, nickel chloride, and a mixture of nickel sulphate and nickel chloride, in the presence of a compound soluble in the acid nickel solution and containing the group  $-\text{SO}_2\text{N}-$  and in the presence of a zinc salt in an amount corresponding to less than about .3 gram zinc per liter of solution.
8. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein a compound containing the group  $-\text{SO}_2\text{N}-$ .
9. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein a compound containing the group  $-\text{SO}_2\text{N}-$  in amounts falling within a range of from .1 gram per liter of solution to saturation.
10. A bath for electrodepositing nickel to obtain a fine grained lustrous deposit comprising an aqueous acid nickel solution comprising essentially boric acid and a material selected from the group consisting of nickel sulphate, nickel chloride, and a mixture of nickel sulphate and nickel chloride, having a pH falling within a range of from about 2 to about 6 electrometric and having dissolved therein a compound containing the group  $-\text{SO}_2\text{N}-$  in amounts falling within a range of from .1 gram per liter of solution to saturation.
11. A method for electrodepositing nickel to obtain a fine grained lustrous deposit comprising the step of electrodepositing nickel from an aqueous acid nickel solution comprising essentially nickel sulphate, nickel chloride and boric acid and containing p-toluene sulphonamide.
12. A method for electrodepositing nickel to obtain a fine grained lustrous deposit comprising the step of electrodepositing nickel from an aqueous acid nickel solution comprising essentially nickel sulphate, nickel chloride and boric acid and containing p-toluene sulphonamide.

acid and containing p-toluene sulphonchloramide.

13. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, having a pH falling within a range of from about 2 to about 6 electrometric in the presence of a compound containing the group



which compound is soluble in the solution and has a concentration in the solution falling within a range of .1 gram per liter of solution to saturation, and a small amount of a metal from the group consisting of zinc and cadmium.

14. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, having a pH falling within a range of from about 2 to about 6 electrometric in the presence of a compound containing the group  $-\text{SO}_2\text{N}=$ , which compound is soluble in the solution and has a concentration in the solution falling within a range of .1 gram per liter of solution to saturation, and maintaining the temperature of the solution within a range from about 15° C. to about 55° C., and a small amount of a metal from the group consisting of zinc and cadmium.

15. A method for electrodepositing nickel to obtain a fine grained lustrous deposit comprising the step of electrodepositing nickel from an aqueous acid nickel solution comprising essentially boric acid and a material selected from the group consisting of nickel sulphate, nickel chloride, and a mixture of nickel sulphate and nickel chloride, having a pH falling within a range of from about 2 to about 6 electrometric in the presence of a compound containing the group  $-\text{SO}_2\text{N}=$ , which compound is soluble in the solution and has a concentration in the solution falling within a range of .1 gram per liter of solution to saturation, and maintaining the temperature of the solution within a range from about 15° C. to about 55° C., and a small amount of a metal from the group consisting of zinc and cadmium.

16. A bath for electrodepositing nickel to obtain a fine grained lustrous deposit comprising an aqueous acid nickel solution comprising essentially nickel sulphate, nickel chloride and boric acid having a pH falling within a range of from about 4 to about 5.3 electrometric and having dissolved therein a compound containing the group  $-\text{SO}_2\text{N}=$  in amounts falling within a range of from .1 gram per liter of solution to saturation, and a small amount of a metal from the group consisting of zinc and cadmium.

17. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride,

in the presence of a compound soluble in the acid nickel solution and containing the group



18. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, in the presence of a compound containing the group



which compound is soluble in the solution and has a concentration in the acid nickel solution falling within the range of from .1 gram per liter of solution to saturation.

19. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein a compound containing the group



20. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein a compound containing the group



in amounts falling within a range of from .1 gram per liter of solution to saturation.

21. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, in the presence of an aromatic compound soluble in the acid nickel solution and containing the group  $-\text{SO}_2\text{N}=$ .

22. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, in the presence of an aromatic compound containing the group  $-\text{SO}_2\text{N}=$ , which compound has a concentration in the acid nickel solution falling within the range from .1 gram per liter of solution to saturation.

23. A method for electrodepositing nickel to obtain a fine grained lustrous deposit comprising the step of electrodepositing nickel from an

5 aqueous acid nickel solution comprising essentially a material selected from the group consisting of nickel sulphate, nickel chloride, and a mixture of nickel sulphate and nickel chloride, having a pH falling within a range of from about 2 to about 6 electrometric in the presence of an aromatic compound containing the group  $-\text{SO}_2\text{N}-$ , which compound is soluble in the solution and has a concentration in the solution 10 falling within a range of .1 gram per liter of solution to saturation.

15 24. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein an aromatic compound containing the group  $-\text{SO}_2\text{N}-$ .

20 25. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein an aromatic compound containing the group  $-\text{SO}_2\text{N}-$  in amounts falling within a range of from .1 gram per liter of solution to saturation.

25 30 26. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, and a material selected from the group consisting of boric acid, formic acid, furoic acid and fluoboric acid, having a pH falling within a range of from about 2 to about 6 electrometric in the presence of a compound containing the group



35 45 which compound is soluble in the solution and has a concentration in the solution falling within a range of .1 gram per liter of solution to saturation, and a small amount of a metal from the group consisting of zinc and cadmium.

50 55 27. A bath for electrodepositing nickel to obtain a fine grained lustrous deposit comprising an aqueous acid nickel solution comprising essentially a material selected from the group consisting of nickel sulphate, nickel chloride, and a mixture of nickel sulphate and nickel chloride, having dissolved therein a compound containing the group



and a small amount of a metal from the group consisting of zinc and cadmium.

5 28. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, and a material selected from the group consisting of boric acid, formic acid, furoic acid and fluoboric acid, in the presence of a compound soluble in the acid nickel solution and containing the group  $-\text{SO}_2\text{N}-$ .

10 15 29. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, and a material selected from the group consisting of boric acid, formic acid, furoic acid and fluoboric acid, in the presence of an aromatic compound containing the group  $-\text{SO}_2\text{N}-$ , which compound is soluble in the solution and has a concentration in the acid nickel solution falling within the range of from .1 gram per liter of solution to saturation.

20 25 30 35 30. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, and a material selected from the group consisting of boric acid, formic acid, furoic acid and fluoboric acid, in the presence of a compound soluble in the acid nickel solution and containing the group



40 45 31. A method for electrodepositing nickel to obtain a fine grained lustrous deposit comprising the step of electrodepositing nickel from an aqueous acid nickel solution comprising essentially a material selected from the group consisting of nickel sulphate, nickel chloride, and a mixture of nickel sulphate and nickel chloride, and a material selected from the group consisting of boric acid, formic acid, furoic acid and fluoboric acid, in the presence of an aromatic compound soluble in the acid nickel solution and containing the group  $-\text{SO}_2\text{N}-$ .

HENRY BROWN.